

## UNITED STATES PATENT OFFICE

2,402,863

## BLENDED GASOLINE

Hilbert H. Zuidema, Edwardsville, and John E. Mital, Alton, Ill., assignors to Shell Development Company, San Francisco, Calif., a corporation of Delaware

No Drawing. Application November 13, 1943,  
Serial No. 510,226

9 Claims. (Cl. 44—62)

1

This invention relates to blended gasolines of improved stability, and is more particularly concerned with leaded gasolines containing up to about 10% and preferably between about 1/2 and 7% alicyclic olefines preferably containing a cyclohexene ring.

Cracked gasolines have always been considered relatively unstable in contrast to straight run gasoline because the former contain olefines while the latter do not. This difference in stability has been known to be further aggravated by the presence of tetra ethyl lead, tetra ethyl lead blends of cracked gasolines being notoriously unstable unless strongly inhibited with an inhibitor serving to stabilize both the olefines as well as the tetra ethyl lead.

We have now discovered that the presence of cyclic olefines, preferably containing a C<sub>6</sub> cyclo olefine ring, in amounts up to about 10% in various gasolines tends to stabilize the gasoline rather than render it unstable. Cyclic olefines as herein defined are alicyclic hydrocarbons containing an olefinic double bond in the ring. Our invention therefore comprises adding to a gasoline containing little or no cyclic olefines, whether it be straight run, cracked, or synthesized, cyclic olefines in amounts such that the concentration of cyclic olefines in the final blend is not above about 10% by volume and preferably between about 1/2 and 7%. The blended gasoline may contain tetra ethyl lead in the usual amounts, e. g. up to about 5 or 6 cc./gal., and preferably should contain effective amounts of an oxidation inhibitor. The added cyclo olefines should boil within gasoline boiling range, and may, if desired, contain (preferably not more than one) olefinic double bond other than the one in the ring.

Possible sources of alicyclic olefines include the terpenes. Other cyclic olefines may be prepared by various syntheses, such as partial dehydrogenation of naphthalenes. Individual cyclic olefines suitable for the purpose include cyclohexene, methyl cyclohexene, dimethyl cyclohexene, trimethyl cyclohexene, ethyl cyclohexene, methyl ethyl cyclohexene, etc.; terpenes, such as di-limonene (citrene), d-l-limonene, (dipentene), terpinolene, alpha, beta or gamma terpinene, phelandrene; dihydroterpenes such as menthene, carvomenthene, etc.; cyclopentene, methyl cyclopentene, dimethylcyclopentene, ethyl cyclopentene, etc.

Usually the content of cyclo olefines in gasolines is quite low, below about 1/2%. Therefore, the addition of cyclo olefines generally results in some improvement.

Different types of oxidation inhibitors affect the stability of the blended gasoline somewhat differently. Especially useful are aromatic amino

inhibitors such as those based on paraphenylenediamine, para amino phenol and alpha naphthylamine, etc. Examples of such inhibitors are the N,N'dibutyl para phenylene diamine, benzyl para amino phenol, phenyl alpha naphthylamine. Other inhibitors such as the purely phenolic inhibitors, as for example 2,4-dimethyl 6-tertiary butyl phenol or 4-methyl 2,6-ditertiary butyl phenol, etc., while enhancing the stability of our blended gasolines are not quite as effective as those mentioned above.

The effect of various olefines, both cyclic and aliphatic, on the induction periods of an alkylate gasoline containing 4 cc. tetra ethyl lead per gallon, being itself substantially free of olefines, is demonstrated in the tables below:

Table I

| Olefine                | Per cent added | Induction period hours (100 p. s. i. O <sub>2</sub> at 100° C.) |                                         |
|------------------------|----------------|-----------------------------------------------------------------|-----------------------------------------|
|                        |                | Uninhibited                                                     | 0.005% N,N'dibutyl paraphenylenediamine |
| None                   |                | 5.9                                                             | 23.0                                    |
| Cyclohexene            | 1/2            | 18.0                                                            | 41.0                                    |
|                        | 2              | 3.8                                                             | 96+                                     |
|                        | 5              |                                                                 | 98+                                     |
|                        | 10             |                                                                 | 58.5                                    |
| Dipentene <sup>1</sup> | 1/2            | 20.2                                                            | 90+                                     |
|                        | 1              | 22.2                                                            | 90.0                                    |
|                        | 2              | 17.5                                                            | 90+                                     |
|                        | 10             |                                                                 | 21.5                                    |
| Mixed amylenes         | 2 1/2          |                                                                 | 8.4                                     |
|                        | 10             |                                                                 | 5.6                                     |
| Di-isobutylene         | 1/2            | 5.6                                                             | 23.1                                    |
|                        | 2              | 5.9                                                             | 21.2                                    |
|                        | 10             | 5.2                                                             | 22.4                                    |

<sup>1</sup> d, l-Limonene.

The effect of cyclic and aliphatic olefines respectively on gum time, i. e. the time required to form 5 mg. A. S. T. M. gum upon exposure to 100 lbs./sq. in. oxygen at 100° C. of an alkylate gasoline containing 4 cc. tetra ethyl lead and 0.005% of N,N'dibutyl para phenylene diamine is demonstrated below:

Table II

| 50             | Olefine | Percent added | 5 mg. A. S. T. M. gum time, hours |
|----------------|---------|---------------|-----------------------------------|
| None           |         |               |                                   |
| Cyclohexene    | 1/2     |               | 23.3                              |
|                | 2       |               | 40.0                              |
|                | 5       |               | 96+                               |
|                | 10      |               | 58.5                              |
| Di-isobutylene | 1/2     |               | 22.0                              |
|                | 2       |               | 21.4                              |
|                | 5       |               | 22.4                              |
|                | 10      |               | 22.4                              |

60 The amount of the oxidation inhibitors em-

ployed in our gasoline do not differ from those customarily employed. Thus these amounts are normally less than .1% and usually between .001 and .01%.

Other additives such as aniline, methyl aniline, toluidene, xylidene, cymidene, etc., or branched chain ethers as methyl tertiary butyl ether and others, as are sometimes used to increase anti-knock properties, volatility, etc., may also be present.

The invention is applicable to automotive gasolines as well as aviation gasolines.

We claim as our invention:

1. A naturally unstable gasoline stabilized against oxidation by the addition of a cycloolefin boiling within gasoline boiling range and possessing a single olefinic double bond in the naphthenic ring, in an amount such that the cycloolefin content of the resulting blend is about  $\frac{1}{2}\%$ .

2. A naturally unstable gasoline stabilized against oxidation by the addition of a C<sub>8</sub> cycloolefin boiling within gasoline boiling range and possessing a single double bond in the ring, in an amount such that the cycloolefin content of the resulting blend is about  $\frac{1}{2}\%$ .

3. A naturally unstable gasoline stabilized against oxidation by the addition of a cyclohexene boiling within gasoline boiling range, in an amount such that the cycloolefin content of the resulting blend is about  $\frac{1}{2}\%$ .

4. A naturally unstable gasoline stabilized

against oxidation by the addition of a terpene boiling within gasoline boiling range and possessing a single double bond in the ring, in an amount such that the cycloolefin content of the resulting blend is about  $\frac{1}{2}\%$ .

5. A cracked, unstable gasoline stabilized against oxidation by the addition of a cycloolefin boiling within gasoline boiling range and possessing a single double bond in the ring, in an amount such that the cycloolefin content of the resulting blend is about  $\frac{1}{2}\%$ .

6. Method of improving the oxidation stability of a naturally unstable gasoline subject to rapid oxidation, comprising adding to said gasoline a cycloolefin boiling within gasoline boiling range and possessing a single double bond in the ring, in an amount such that the cycloolefin content of the resulting blend is about  $\frac{1}{2}\%$ .

7. A composition comprising a naturally unstable gasoline stabilized against oxidation by the addition of an aromatic amino oxidation inhibitor and of between about  $\frac{1}{2}\%$  and 10% of a cycloolefin boiling within the gasoline boiling range and possessing a single double bond in the ring.

8. A composition according to claim 7, wherein the cycloolefin content is below about 7%.

9. A composition according to claim 7, wherein the cycloolefin content is in the neighborhood of about  $\frac{1}{2}\%$ .

HILBERT H. ZUIDEMA.  
JOHN E. MITAL.